

## UNITED STATES PATENT OFFICE

2,247,280

## STABILIZING FATTY COMPOSITIONS

George D. Martin, Nitro, W. Va., assignor to Monsanto Chemical Company, St. Louis, Mo., a corporation of Delaware

No Drawing. Application July 21, 1939,  
Serial No. 285,767

6 Claims. (CL 23—250)

This invention relates to the treatment of oils containing a fatty component and more particularly to the treatment of animal, vegetable and fish oils for the purpose of inhibiting rancidity and other undesirable effects associated therewith.

Animal, vegetable, fish and the like oils are fatty acid esters, as for example fatty acid glycerides. As is well known, oils of this type are subject to changes characterized by the formation of malodorous products which render them unsuitable for foodstuffs and for many other purposes. This condition is commonly referred to as rancidity. Where the fatty acid components of the oil comprise an unsaturated constituent the susceptibility to rancidity is materially enhanced. Rancidity is believed to result from the formation of aldehydes, ketones, peroxides and similar oxidative degradation products of the oil and is usually further characterized by a bleaching action due to the peroxide content. For example olive oil is normally the familiar light golden color whereas the rancid product is colorless and possesses a decidedly unpleasant taste and odor. The transformation to the latter condition is accelerated by heat, light and various chemical agents and in general special precautions are necessary in handling and storing vegetable, animal and fish oils, especially where intended for human consumption.

It is an object of this invention to stabilize vegetable, animal, fish and the like oils and more particularly to prevent the development of rancidity.

One of the specific objects of this invention is to provide a rancidity inhibiting or retarding agent to be incorporated with the oil which is to be stabilized. A further object is to provide an oil composition stabilized against the development of rancidity. Other and further objects will be hereinafter shown.

In accordance with present invention it has been discovered that the neutral phosphates of polyhydric phenols are highly effective stabilizers of oils containing a fatty component. Esters of inorganic acids in which the inorganic acid nucleus is completely esterified, i. e. no replaceable hydrogen remains, are commonly termed "neutral esters" and it is in this sense that the term "neutral" is herein employed.

The preferred esters may be prepared by known methods from suitable esterifying agents such as  $P_2O_5$  and  $POCl_3$  and a polyhydric phenol. Neutral phosphates derived from catechol, tertiary amyl catechol, tertiary butyl catechol, chlor catechol, pyrogallol, resorcinol, hydroquinone, hydroxy hydroquinone, 3,4 dioxy biphenyl, p,p' dioxy biphenyl, 3,4,4' trioxy biphenyl, 1,2 dioxy naphthalene, 1,5 dioxy naphthalene and the like are included within the scope of this invention.

Typical examples of the preferred class of stabilizers comprise tri o-phenylene phosphate of the formula



10 Tri(4-tertiary butyl o-phenylene) phosphate; tri(4-tertiary amyl o-phenylene) phosphate; tri(4-chlor o-phenylene) phosphate; tri(4-phenyl o-phenylene) phosphate; tri o-naphthylene phosphate; tri(3-hydroxy o-phenylene) phosphate; tri(4-hydroxy o-phenylene) phosphate; tri(5-hydroxy 1-naphthyl) phosphate and equivalents and analogues thereof.

15 The following is a typical method employed in evaluating stabilizers of oils subject to the development of rancidity:

20 A convenient quantity, for example 0.05% to 1.0% by weight of the stabilizing agent is incorporated in an oil tending to develop rancidity. The treated oil is heated in an open flask for several days in an oven maintained at 50° C. 25 After various intervals of time the aged samples are tested in a manner analogous to that described by D. H. Wheeler, Oil and Soap, Vol. 9, page 93, 1932. Thus, five grams of the oil are dissolved in 50 c. c. of solvent mixture (60 percent of glacial acetic acid, 40 percent of chloroform) and 1 c. c. of saturated potassium iodide solution added. After exactly one minute from the time of the addition of potassium iodide, 100 30 c. c. of water are added and the liberated iodine titrated with 0.01N sodium thiosulfate, employing starch as indicator. The titration in cubic centimeters is a measure of the peroxide formation and consequently a measure of the stability of the oil. The so called "peroxide number" 35 which is the usual basis of comparison is defined by Wheeler according to the equation

$$M = \frac{T \times N \times 500}{W}$$

40 where W is the weight of the oil and T is the milliliters of thiosulfate of normality N. M is thus the millimols of peroxide per kilogram or the "peroxide number." (See also C. H. Lee, Rancidity in Edible Fats, page 108.) Obviously where a 5 gram sample of oil is titrated with .01N thiosulfate the milliliters required give the peroxide number directly.

45 The following are specific embodiments of the invention showing the useful and valuable properties of the preferred class of stabilizers and are to be understood as illustrative of the invention but in nowise limitative thereof.

50 A small proportion, 0.1% of the stabilizing agent, was incorporated into an unstable oil. The peroxide number was determined as described above and compared with that of the

untreated oil. Typical results obtained upon testing the preferred class of neutral esters are set forth below:

| Cottonseed oil stabilizing agent    | Peroxide number after 30 days aging |
|-------------------------------------|-------------------------------------|
| Tri(4-hydroxy o-phenylene)phosphate | 6.0                                 |
| Tri(3-hydroxy o-phenylene)phosphate | 2.0                                 |
| Tri(4-phenyl o-phenylene)phosphate  | 1.0                                 |
| Tri(5-hydroxy 1-naphthyl)phosphate  | 0.5                                 |
| Blank                               | 390.0                               |

As further illustrative of the desirable properties of the preferred class of stabilizers, the peroxide numbers of typical oils stabilized by the addition of 0.1% of tri(o-phenylene) phosphate as compared with the peroxide number of the untreated oil (Blank) are given below.

| Oil                | Peroxide numbers after aging for— |         |         |         |         |         |
|--------------------|-----------------------------------|---------|---------|---------|---------|---------|
|                    | 10 days                           | 11 days | 24 days | 32 days | 38 days | 46 days |
| Cottonseed         | 8.5                               |         | 10.8    | 9.5     |         |         |
| Blank (cottonseed) | 62.5                              |         | 180.0   |         |         |         |
| Olive              | 1.1                               |         | 1.1     | 0.0     |         |         |
| Blank (olive)      | 28.0                              |         | 106.0   | 145.0   |         |         |
| Sardine            | 7.0                               |         |         |         |         |         |
| Blank (sardine)    | 30.5                              |         |         |         | 2.7     | 3.8     |
| Oleic acid         |                                   | 3.5     |         |         | 14.0    | 24.6    |
| Blank (oleic acid) |                                   | 12.7    |         |         |         |         |

The following data show the peroxide numbers of oleic acid stabilized with 0.1% or tri(4-tertiary amyl o-phenylene) phosphate as compared with the untreated product.

|                 | Peroxide numbers after aging for— |         |         |
|-----------------|-----------------------------------|---------|---------|
|                 | 21 days                           | 34 days | 53 days |
| Treated product | 2.7                               | 1.4     | 5.0     |
| Blank           | 21.0                              | 24.0    | 29.7    |

From the data set forth above it is shown that the preferred stabilizing agents possess exceptional rancidity inhibiting properties when incorporated in unstable oils, as for example animal, vegetable and fish oils.

The amount of stabilizing agent which may be added to an unstable oil may be varied within wide limits but in general it will be found that good results may be obtained by adding, upon a weight basis, from 0.01% to 1.0% of the stabilizing agent.

Other methods of testing the stability of unstable oils than those specifically disclosed may be employed as is well known to those skilled in the art to which the present invention pertains.

The present invention is limited solely by the following claims attached hereto as part of the specification.

20. What is claimed is:

1. A fatty oil having incorporated therein a neutral phosphate of a polyhydric phenol in an amount sufficient to preserve said fatty oil.

25. 2. A fatty oil having incorporated therein a tri (o-arylene) phosphate in an amount sufficient to preserve said fatty oil.

3. A fatty oil having incorporated therein a tri (o-phenylene) phosphate in an amount sufficient to preserve said fatty oil.

30. 4. A fatty oil having incorporated therein tri (4-tertiary amyl o-phenylene) phosphate in an amount sufficient to preserve said fatty oil.

5. A fatty oil having incorporated therein tri (4-hydroxy 1-naphthyl) phosphate in an amount sufficient to preserve said fatty oil.

35. 6. A fatty oil having incorporated therein from 0.01% to 1.0% of a neutral phosphate of a polyhydric phenol.

40. GEORGE D. MARTIN.